

June 9, 1925.

1,541,596

F. SKAUPY ET AL

FILAMENT FOR INCANDESCENT LAMPS OR OTHER VACUUM APPARATUS

Filed Nov. 3, 1924

Fig. 1.



Fig. 2.



Fig. 3.



Inventors:

Franz Skaupy,

Fritz Koref,

by *Maxwell J. L.*  
Their Attorney.

## UNITED STATES PATENT OFFICE.

FRANZ SKAUPY AND FRITZ KOREF, OF BERLIN, GERMANY, ASSIGNEES TO GENERAL ELECTRIC COMPANY, A CORPORATION OF NEW YORK.

## FILAMENT FOR INCANDESCENT LAMPS OR OTHER VACUUM APPARATUS.

Application filed November 3, 1924. Serial No. 747,573.

To all whom it may concern:

Be it known that we, FRANZ SKAUPY and FRITZ KOREF, citizens, respectively, of Austria and of Germany, residing at Berlin, 5 Germany, have invented certain new and useful Improvement. Filaments for Incandescent Lamps or Other Vacuum Apparatus (for which we have filed applications in Germany August 29, 1923, P. 46,748 10 VIII/21f (withdrawn); filed in Japan December 8, 1923, No. 1,574; filed in Great Britain February 27, 1924, No. 5,060/24 (abandoned); an amended case filed in Germany April 7, 1924, P. 48,128 VIII/21f2), 15 of which the following is a specification.

Our invention relates to filaments for incandescent lamps or other vacuum devices and the process of its manufacture. More particularly, however, it relates to filaments 20 of the macro-crystal or uni-crystal type.

The details of our invention are herein-after more fully set forth and claimed, reference being had to the accompanying drawing in which Fig. 1 is a diagrammatic representation of a cross-section of the known 25 form of a filament; Fig. 2 is a diagrammatic representation of a cross-section of a new form of filament; Fig. 3 is a diagrammatic representation of a cross-section of 30 another form of filament.

Experiments which have been made with these filaments have demonstrated that the filaments continue to decrease in size the longer they are burned due to the atomization 35 or evaporation of the material. Fig. 1 is the diagrammatic representation of the cross-section of a filament of uni-crystal type which initially is round and which gradually decreases in size, assuming a 40 polygonal cross-section or one with curved surfaces, as indicated by the heavy line  $a-a$  in this figure. In this manner the filament assumes after a period of operation a polygonal shape and the number of surfaces 45 formed depends upon the positions of the long crystals with respect to the axis of the filament. In this manner and after a period of operation also a polygonal filament 50 can be obtained which has more than four lateral surfaces, six or eight for instance. The polygonal or semi-polygonal

cross-section is due to the fact that the evaporation does not occur at the same rate over the surface of the filament. According to certain crystallographic laws the 55 minimum volatilization takes place along the line  $b-b$  where the edges  $b$  form themselves. On the other hand, the most severe volatilization takes place along the central part of the surface between the two edges. 60 As soon as the volatilization of the round filament has reached a sufficient stage, as for instance as far as the surface indicated by the line  $a-a$ , the volatilization proceeds nearly evenly along the entire surface of the filament. As the volatilization 65 continues the configuration of the cross-section remains approximately the same and for this reason a much greater amount of material is disintegrated within the same time 70 than at the beginning, as indicated by the fact that the cross-section indicated by the outline  $a-a$  is reduced to that indicated by the outline  $c-c$ . The more the cross-section of the filament varies from the 75 original shape the more pronounced becomes the volatilization and therefore the blackening of the lamp. However, in practice the life of the filament ceases as soon as the polygonal cross-section, which remains 80 constant in shape, is obtained.

According to the invention this fact is made use of in manufacturing filaments which, during the time which the round cross-section changes into the final polygonal or curve-polygonal cross-section, do not evaporate or atomize to such an extent as the crystal filaments with round cross-sections. According to the invention the 85 filaments (or crystals comprising them 90 which may consist of metals of high melting points such as tungsten or other refractory metals such as oxides or nitrides) are given, for the purpose in view, such a polygonal cross-section that their lateral area 95 consists entirely or mainly of slightly curved surfaces which disintegrate or atomize as slowly as possible, and which to this end form an angle with the surfaces, or 100 surface, that form themselves automatically during the process of evaporation.

With this new polygonal shape of fila-

ment, the part at or nearly at edges of the faces evaporate at a maximum rate whereas the more centrally located parts of the faces are far less subject to evaporation or 5 atomization. As can be seen from Fig. 2 much more time will elapse with the new shape than with the former one until the filament will assume the permanent form of 10 cross-section indicated at heavy lines  $f-f$ , thus, the blackening of the bulb caused by 15 evaporation or atomization is prevented and the longevity of the filament is increased.

To obtain the desired results the faces of 20 the polygonal filament can be slightly curved instead of being straight, as shown in Fig. 2. The lateral area of the filament need not be composed exclusively of faces with minimum rate of evaporation, it is sufficient when the latter at least predominate on the surface. For instance, the filament can have a cross-section such as indicated in Fig. 3 where  $g$  indicates faces of 25 minimum wear and  $h$  faces where the wear is more pronounced.

25 In order to manufacture the new filament, an ordinary round filament may be used to start with which by a preliminary heat treatment is converted into one single crystal or into a number of crystals forming 30 the entire cross-section of the filament. After that the crystal filament is heated in a liquid mixture or in a gaseous atmosphere containing the constituent parts of the filament. In this manner, the filament increases 35 in size after a certain lapse of time because of the material deposited from the liquid or from the gaseous atmosphere and it assumes automatically a polygonal cross-section. It is thus possible to convert wire-shaped round tungsten crystals when heating 40 them in a mixture of hydrogen and tungsten hexachloride into such a polygonal cross-section. Strange to say, it has been found, that a round cylindrical filament grows 45 in a liquid mixture or in the gaseous atmosphere in such a manner that the surfaces that are produced are not parallel but are at an angle to those obtaining during 50 the process of disintegration. In this manner the faces of the filament coincide with the planes where the evaporation is least pronounced.

55 Filaments of the desired cross-section can also be obtained by causing the filament to become reduced before use, not by evaporation or by atomization, but in the following manner: It has been found that the volatilization of filaments causes them to assume quite different shapes, depending upon the 60 nature of the solvent utilized in the process. For instance, with the tungsten crystals an acid solvent causes a different formation during the reduction than an alkaline solvent. With such corrosive solvents and substances or gases, filaments are obtained 65

whose plane or slightly curved surfaces form an angle with the faces that are created when the filament evaporates or atomizes.

Finally, it is possible with sufficiently strong filaments consisting of a single or of 70 few macro-crystals, especially oxide crystal filaments, to obtain the desired faces by means of mechanical processes such as grinding. In order to obtain the right position of the surfaces that are to be ground, 75 it is necessary to previously etch slightly the crystal or crystals at any place, preferably at one end. In this manner, not only the right position but also the shape of the crystal or crystals before the subsequent 80 grinding can be determined.

What we claim as new and desire to secure by Letters Patent of the United States, is:—

1. A macro-crystal filament of a refractory metal having a polygonal cross-section 85 in its initial form, which filament when heated reduces to a filament having a second and different form having also a polygonal cross-section, the filament in the first form having one of its sides in a position 90 at an angle to the position of any of the sides of the filament in its second form.

2. A filament of a refractory metal for producing radiation, said filaments having 95 a polygonal cross-section which when subjected to an electric current reduces to a filament having a different polygonal cross-section, the filament in the first instance having sides in a position at an angle to the 100 sides of the filament in the second instance.

3. A filament of a refractory metal having 105 a polygonal cross-section, said filament so constructed that the central longitudinal zone of one of the surfaces has a minimum rate of evaporation when heated.

4. A filament of a refractory metal having 110 an internal polygonal structure and an external polygonal structure angularly displaced about the longitudinal axis of the filament.

5. A filament of a refractory metal for transmitting radiant energy, said filament having an external polyhedral structure and an internal polyhedral structure, one of the structures having faces sloping with respect 115 to faces of the other structure.

6. A filament of a refractory metal for transmitting radiant energy, said filament having an external polyhedral structure and an internal polyhedral structure, one of the structures having faces sloping with respect 120 to faces of the other structure, the apex lines forming the intersection of adjacent faces of the internal structure extending each parallel to and in proximity of the central longitudinal zone of one of the faces of the external structure.

7. A filament of a refractory metal for transmitting radiant energy, said filament 130 having an external polyhedral structure and

an internal polyhedral structure, one of the structures having faces sloping with respect to faces of the other structure, the faces of the structures extending in the same direction with the axis of the filament.

8. A macro-crystal filament for a device for radiating energy having a polygonal

cross-section and having surfaces with a relatively low rate of evaporation.

In witness whereof, we have hereunto set our hands this 11th day of October, 1924.

FRANZ SKAUPY.  
FRITZ KOREF.